

# United States Patent

[19]

Wincklhofer et al.

[11] 3,873,353

[45] Mar. 25, 1975

[54] ANTISTATIC FIBER

[75] Inventors: **Robert Charles Wincklhofer**,  
Richmond; **Judd Leonard Schwartz**,  
Chester, both of Va.

[73] Assignee: **Allied Chemical Corporation**, New  
York, N.Y.

[22] Filed: **Mar. 5, 1973**

[21] Appl. No.: **337,777**

[52] U.S. Cl..... **117/138.8 A, 117/138.8 D,**  
**117/138.8 F, 117/138.8 N,**  
**117/139.5 A**

[51] Int. Cl..... **B44d 1/22**

[58] Field of Search ..... **117/139.5 A, 139.5 CQ,**  
**117/138.8 N, 138.8 F, 138.8 D, 47 R, 138.8**  
**A; 260/857 PE**

## [56] References Cited

### UNITED STATES PATENTS

2,727,004 12/1955 Cohen ..... **117/139.5 CQ**  
2,974,066 3/1961 Macura et al..... **117/139.5 A**

|           |        |                   |              |
|-----------|--------|-------------------|--------------|
| 3,333,983 | 8/1967 | Sellet .....      | 117/139.5 UA |
| 3,470,267 | 9/1969 | Litt et al.....   | 117/138.8 N  |
| 3,657,386 | 4/1972 | Weodon et al..... | 260/77.5 A   |

Primary Examiner—William D. Martin

Assistant Examiner—Theodore G. Davis

Attorney, Agent, or Firm—Fred L. Kelly

[57]

## ABSTRACT

An improved antistatic fiber of polyamide, polyester, polyurea, polyurethane or polysulfonamide is prepared by uniformly dispersing an antistatic additive consisting of a chain-extended propylene oxide-ethylene oxide copolymer based on a diamine, in the fiber-forming polymer, forming the fiber by conventional methods, then applying to the fiber a coating of the antistatic additive. The improved antistatic fiber is especially useful for carpet manufacture. In carpet use, the antistatic additive included in the fiber improves with age, whereas the additive externally added is gradually abraded off in use; the net result is a relatively stable antistatic capability.

4 Claims, No Drawings

## ANTISTATIC FIBER

## REFERENCE TO RELATED APPLICATIONS

This application is related to U.S. application Ser. No. 294,971, filed Oct. 11, 1972 by Gene C. Weedon and Lamberto Crescentini.

## BACKGROUND OF THE INVENTION

This invention relates to a process for the melt-spinning of a filamentary structure from a synthetic polymer such as polyamide, polyester, polyurea, polyurethane or polysulfonamide. More particularly, it is concerned with an improved process for the formation of an improved antistatic filament, yarn or the like by melt-spinning a synthetic linear fiber-forming polymer containing an antistatic additive, and thereafter treating the fibrous structure with an antistatic composition to improve the antistatic properties.

It has been suggested that the utility of synthetic fibers could be increased and their properties, in particular their antistatic properties, could be improved if a polyalkylene ether of high molecular weight is included in the polymer. More specifically, it is disclosed in U.S. Pat. No. 3,475,898 to Magat and Sharkey to use poly(ethylene-propylene)ether glycols for this purpose. More recently, U.S. Pat. No. 3,657,386 discloses that certain propylene oxide-ethylene oxide copolymers based on ethylene diamine are useful in preparation of an antistatic fiber of polyamide. The present invention is an improvement upon the invention disclosed in U.S. Pat. No. 3,657,386.

## SUMMARY OF THE INVENTION

Applicants have discovered that a superior antistatic fiber of polyamide, polyester, polyurea, polyurethane or polysulfonamide can be prepared by uniformly dispersing in the fiber-forming polymer an antistatic additive consisting of a chain-extended tetrol based on a diamine, forming the fiber by conventional methods, and then applying to the fiber a coating of the antistatic additive. This chain-extended tetrol based on a diamine is a predominantly branched chain-extended polymer of the reaction product of a tetrol compound represented by the formula:



where  $a$ ,  $b$ ,  $c$ ,  $d$ ,  $w$ ,  $x$ ,  $y$ , and  $z$  are each a whole number and  $\text{R}$  is a difunctional radical from a hydrocarbon containing 1 to 13 carbon atoms, preferably a lower alkyl aliphatic hydrocarbon containing 1 to 6 carbon atoms, and at least one compound selected from the group consisting of diepoxides and compounds which yield the following divalent radicals:



where  $\text{R}'$  is a difunctional radical derived from aromatic, heterocyclic, cycloaliphatic or aliphatic hydrocarbons or combinations of them. Preferably, the ethylene oxide moiety makes up 10 to 90% of the molecular weight of the tetrol compound. The improved antistatic fiber is especially useful for carpet manufacture.

In carpet use, the antistatic additive included in the fiber improves with age, whereas the additive externally added is gradually abraded off in use; the net result is a relatively stable antistatic capability.

The chain-extended compound is added to the polymer in amounts from about 1 to about 12% by weight, preferably about 2 to about 10% by weight. The yarn is preferably coated with between about 0.05 and about 15 6% by weight, preferably 0.1 to 3% by weight, based on the finished yarn, of the chain-extended compound. The chain-extended compound is preferably applied to the yarn in the form of a solution in a suitable solvent such as water, benzene, or ethyl alcohol; concentrations between about 0.1 and about 10% are suitable. The coated yarn may be heated, if desired, to cause volatilization of the solvent.

The tetrol compound which is chain-extended for use as an antistatic additive in this invention is fully described in U.S. Pat. No. 2,979,528 to Lundsted, assignor to Wyandotte. These tetrol compounds are commercially available as tetronic series block copolymers having molecular weights between 1,650 and over 26,000. This series varies in length of poly(oxyethylene) chain and poly(oxypropylene) chain. A 3 and 4 digit code number indicates the molecular composition. When four digits are employed, the first two explain the average molecular weight of the hydrophobe (poly(oxypropylene)) (oxypropylene) branches on the alkylene-diamine. When three digits are used only the first number serves this purpose. The last digit of each code number represents the weight percentage of hydrophilic (poly(oxyethylene)) units to the nearest 10%. The tetrol compounds in the examples are described this way.

As diamines upon which the tetrols are based, in addition to ethylene diamine, diamines of the hydrocarbon containing 1 to 13 carbon atoms, preferably the lower alkyl diamines, where the lower alkyl radical

45

contains 1-6 carbon atoms, can be used.

The polyepoxy coupled compounds can be prepared by the method taught in British Pat. No. 793,915, Example I. The other classes of compound can be similarly prepared, as in Example 10 in U.S. Pat. No 60 3,009,884.

Typical of the acids and their esters to provide the chain-extending difunctional radical are the dialkyl phthalic, isophthalic or terephthalic esters, such as dimethyl terephthalate and adipic, phthalic, terephthalic, sebacic, glutaric, pimelic, isocinchomeric acids and their esters.

Typical of the polyepoxy compounds which provide the difunctional or divalent compounds, used to chain-extend the tetrols based on diamines, are those poly-

poxy compounds described in British specification No. 793,915 to Union Carbide on page 2, line 48 to line 121 as follows:

"The organic polyepoxy compounds suitable for use in preparing the polymeric products of this invention are organic compounds having as the sole reactive groups under the conditions of this reaction, at least two epoxy groups. By this we mean to exclude compounds containing carboxyl, hydroxyl, phenolic hydroxyl, amino, amido, imido and mercapto groups, which have been found to be reactive under the conditions of this reaction with epoxy groups of the polyepoxy compound or with the hydroxyl groups and alkali metal alcoholate groups of the polyoxyalkylene glycol, and thus will interfere with the desired condensation. These polyepoxy compounds free of such interfering groups can be aliphatic, cycloaliphatic and aromatic, and can contain non-interfering substituent groups such for example as alkyl, aryl, organic ester, phosphate ester, halogen and cyano groups without interfering with the condensation. Olefinic unsaturation in the polyepoxy compound can also be present.

The preferred organic polyepoxy compounds are the aliphatic, cycloaliphatic and aryl substituted aliphatic compounds having as the sole reactive groups under the conditions of the reaction, at least two epoxy groups, and wherein oxygen is present only in oxirane, ether and ester arrangement. Particularly preferred are the diepoxy compounds consisting only of carbon, hydrogen and oxygen, wherein oxygen is present only in oxirane, ether and ester arrangement, and wherein the epoxy groups are terminal groups of an aliphatic or aryl substituted aliphatic compound or where the epoxy group or groups include adjacent carbon atoms of a cycloaliphatic ring. Representative of these preferred compounds are butadiene diepoxide, diglycidyl ether, the diglycidyl ether of 2,2-bis(4-hydroxyphenyl)-propane, 4-vinyl-cyclohexene diepoxide, dicyclopentadiene diepoxide, bis(2,3-epoxycyclopentyl)ether, ethylene glycol bis(3,4-epoxy-methylcyclohexane-carboxylate) and the 3,4-epoxy-methylcyclohexylmethyl 3,4-epoxy-methylcyclohexanecarboxylate.

It is to be understood that the invention is not limited to the foregoing compounds alone and a variety of organic polyepoxy compounds can be used. While it is preferred that the epoxy groups be terminal groups or include adjacent carbon atoms of a cycloaliphatic ring, aliphatic and substituted aliphatic compounds having adjacent carbon atoms of the epoxy group as adjacent intermediate carbon atoms of a linear chain may be used. However, compounds having such internal epoxy groups react somewhat slower compared with those compounds having terminal epoxy groups.

A mixture of two or more polyepoxy compounds can be used in the practice of this invention, or if desired, the polyoxyalkylene glycol can be reacted successively with different polyepoxy compounds to obtain these polymeric products.

These polyepoxy compounds serve both as chain extenders between polyalkylene glycol chains and as cross-linking agents. According to our experience, primary hydroxyl groups of the polyoxyalkylene glycol react preferentially with the epoxy groups to link up the polyglycol chains, creating secondary hydroxyl groups upon opening of the epoxide ring.

Also useful to form chain-extending divalent radicals are the aromatic or aliphatic diisocyanates, having a structure  $OCN-R'-NCO$ , where  $R'$  is defined as above.

5 The antistatic fiber of this invention may also contain conventional fiber additives such as antioxidants, stabilizers, delusterants, dyeing assists, and colorants.

#### DESCRIPTION OF THE PREFERRED EMBODIMENT

10

In order to demonstrate the invention, the following examples are given. They are provided for illustrative purposes only and are not to be construed as limiting the scope of the invention, which is defined by the appended claims. parts and percents are by weight unless otherwise indicated. Parts

15 Following is a list of properties of tetrol compounds identified by Tetronic numbers in the Examples.

20

| Tetronic | Molecular Weight | Brookfield Viscosity at 25°C. (cps) | Pour Point °C. | Melting Point. °C. |
|----------|------------------|-------------------------------------|----------------|--------------------|
| 25 908   | 26,100           | — (solid)                           | —              | 58                 |
| 1,302    | 7,800            | 1,300                               | 13             | liquid at 25       |
| 1,504    | 12,500           | 1,570                               | 18             | liquid at 25       |
| 30 1,506 | 20,000           | — (solid)                           | —              | 50                 |

30

#### EXAMPLE 1

A glass reactor equipped with a heater and stirrer was charged with a mixture of 1,520 grams of  $\epsilon$ -caprolactam and 80 grams of aminocaproic acid. The mixture was then flushed with nitrogen and was stirred and heated to 255°C. over a one hour period at atmospheric pressure to produce a polymerization reaction. The heating and stirring was continued at atmospheric pressure under a nitrogen sweep for an additional four hours in order to complete the polymerization. Nitrogen was then admitted to the glass reactor and a small pressure was maintained while the polymer was extruded from the glass reactor in the form of a polymer ribbon. At this time, 90 grams of antistatic additive was mixed into the polymer, the antistatic additive being the reaction product of Tetronic 1504 and dimethyl terephthalate (DMT) in a 1 to 0.9 mol ratio. This additive is soluble in toluene and water and has a melt viscosity of 10,000 centipoises at 100°C. The antistatic additive was mixed into the polymer by blending molten polymer and antistatic additive in a static mixer to produce a uniform dispersion of antistatic additive in the extrudate. The polymer ribbon was subsequently cooled, pelletized using a Wiley Mill, washed and then dried. The polymer was a white solid having a relative viscosity of about 50 to 60, as determined at a concentration of 11 grams of polymer in 100 ml. of 90 percent formic acid at 25°C. (ASTMD-789-62T).

60

#### EXAMPLE 2

Polymer pellets prepared in accordance with Example 1 and containing the antistatic agent were melted at about 285°C. and then melt extruded under pressure of 1,500 psig to a 70-orifice spinnerette, each of the orifices having a diameter of 0.018 inch to produce a fiber having about 4,500 denier. The fiber was collected at about 1,000 feet per minute and was drawn at

about 4 times the extruded length to produce yarn having a denier of about 1,050. This yarn will hereinafter be called Yarn A. A control yarn containing no antistatic agent was prepared in the same manner as described above. This yarn will hereinafter be called Yarn B.

The yarns were textured using a steam jet and then two-plyed by twisting two ends together with a 1½ S twist. The yarns were tufted into a level loop 20 oz. carpet at about 6.5 stitch rate, about 9/32 to 10/32 inch pile height, dyed and latexed. Static buildup of the carpet was tested by measuring the electrostatic voltage buildup on a person walking with a series of steps on a piece of carpet according to the standard CRI Walk Test for static propensity in carpets, also labeled AATCC 134-1969. Carpet was conditioned at 70°F. at 20 percent relative humidity. Results are shown in the following Table.

| Carpet           | Static Walk Test |
|------------------|------------------|
| Made with Yarn A | 6.1 KV           |
| Made with Yarn B | 14.1 KV          |

### EXAMPLE 3

Carpet samples prepared from Yarn A in accordance with Example 2 were treated as follows to coat the fibers with the antistatic additive of Example 1.

Aqueous solutions of the antistatic additive were prepared at three levels, namely 3, 1 and 0.3% by weight, based on the total weight of the solution. The three solutions were applied to three different samples of the carpet during the "wet-out" phase of the carpet dyeing operation prior to drying of the finished carpet. Sufficient solution was applied to the carpet samples to provide 3, 1 and 0.3% of the antistatic additive as a coating on the fibers of the dried carpet. A control carpet sample was prepared from Yarn A in the same manner except that water was used in place of the solution of antistatic additive. Static buildup of the carpet samples was tested in accordance with the procedure described in Example 2. Results are shown in the following Table.

| Carpet                              | Static Walk Test |
|-------------------------------------|------------------|
| Yarn A with no antistatic coating   | 6.1 KV           |
| Yarn A with 0.3% antistatic coating | <0.5 KV          |
| Yarn A with 1.0% antistatic coating | <0.5 KV          |
| Yarn A with 3.0% antistatic coating | <0.5 KV          |

Similar excellent results were obtained when the antistatic additive used was of similar structure to that described in Example 1 except that the tetrol starting compound was Tetronic 908, Tetronic 1302 or Tetronic 1506.

Additional tests showed that the antistatic additive included in the fiber improved in antistatic capability with age, whereas the antistatic additive externally added was gradually abraded off in use; the net result was a relatively stable antistatic capability.

### EXAMPLE 4

The procedure of Example 1 was followed with a ma-

terial of similar structure to that described except that the DMT/polyether mol ratio was 1.0 and melt viscosity was about 17,500 centipoises at 100°C. Carpet samples prepared, coated with the instant antistatic additive, then tested in accordance with Examples 2 and 3, showed a static build-up of less than 0.5 K.V.

### EXAMPLE 5

A glass reactor equipped with a heater and stirrer was charged with a mixture of 1,520 grams of e-caprolactam and 80 grams of aminocaproic acid. The mixture was then flushed with nitrogen and was stirred and heated to 255°C. over a 1 hour period at atmospheric pressure to produce a polymerization reaction.

15 The heating and stirring was continued at atmospheric pressure under a nitrogen sweep for an additional four hours in order to complete the polymerization. During the last 30 minutes of the polymerization, 60 grams of the antistatic additive of Example 1 was added to the 20 polycaproamide and stirring was continued to thoroughly mix the antistatic agent throughout the polymer. Nitrogen was then admitted to the glass reactor and a small pressure was maintained while the polymer was extruded from the glass reactor in the form of a 25 polymer ribbon. The polymer ribbon was subsequently cooled, pelletized using a Wiley Mill, washed and then dried. The polymer was a white solid having a relative viscosity of about 55 to 60, as determined at a concentration of 11 grams of polymer in 100 ml. of 90 percent 30 formic acid at 25°C. (ASTMD-789-62T).

Carpet samples prepared from this polymer, treated with the instant antistatic additive and tested in accordance with Examples 2 and 3, showed a static build-up of less than 0.5 K.V.

### EXAMPLE 6

A glass reactor equipped with a heater and stirrer was charged with a mixture of 1,520 grams of e-caprolactam, 80 grams of aminocaproic acid, 60 grams 40 of an antistatic additive obtained from the reaction product of Tetronic 1504 and dimethyl terephthalate in a 1 to 0.7 mol ratio. The additive was soluble in water and toluene, and had 1,600 centipoise melt viscosity at 100°C. The mixture was then flushed with nitrogen and was stirred and heated to 255°C. over a 1 hour period at atmospheric pressure to produce a polymerization reaction. The heating and stirring was continued at atmospheric pressure under a nitrogen sweep for an additional 2.3 hours in order to complete the polymerization.

55 Nitrogen was then admitted to the glass reactor and a small pressure was maintained while the polymer was extruded from the glass reactor in the form of a polymer ribbon. The polymer ribbon was subsequently cooled, pelletized using a Wiley Mill, washed and then dried. The polymer was a white solid having a relative viscosity of about 55 to 60, as determined at a concentration of 11 grams of polymer in 100 ml. of 90 percent 50 formic acid at 25°C. (ASTMD-789-62T).

60 Carpet samples prepared from this polymer, treated with the instant antistatic additive, and tested in accordance with Examples 2 and 3, showed a static build-up of less than 0.5 K.V.

### EXAMPLE 7

The procedure was that of Example 6 except that 90 grams of the antistatic additive was used instead of 60

grams. Carpet samples prepared from this polymer, treated with the instant antistatic additive, and tested in accordance with Examples 2 and 3, showed a static build-up of less than 0.5 K.V.

#### EXAMPLE 8

The procedure was that of Example 1 except that 60 grams of an antistatic additive obtained from the reaction of Tetronic 1504 and methylene bis(4-cyclohexyl isocyanate) were used. This material had an ethylene oxide content of about 40% and a diisocyanate/polyether mol ratio of 0.9. Carpet samples prepared from this polymer, treated with the instant antistatic additive, and tested in accordance with Examples 2 and 3, showed a static build-up of less than 0.5 K.V.

#### EXAMPLE 9

The procedure was that of Example 1 except 60 grams of an antistatic material derived from the reac-

By "antistatic" fiber is meant fibers that will pass the cling test and the shuffle test as described in U.S. Pat. No. 3,657,386. By "fiber" is meant multifilament yarn, monofilament, and all the known physical forms of synthetic fibers. By "polyamide" is meant the polymers made by condensation of diamines with dibasic acids or by polymerization of lactams or amino acids, resulting in a synthetic resin characterized by the recurring group —CONH—. By "ethylene oxide moiety" is meant the portion of the chemical molecule —(CH<sub>2</sub>C<sub>2</sub>H<sub>2</sub>O)—.

We claim:

1. An antistatic fiber selected from the group consisting of polyamide, polyester, polyurea, polyurethane, and polysulfonamide, said fiber containing between about 1 and about 12% by weight of an antistatic additive consisting of a predominantly branched, chain-extended polymer of the reaction product of a tetrol compound represented by the formula:



30

where  $a, b, c, d, w, x, y$ , and  $z$  are each a whole number and  $R$  is a difunctional radical from a hydrocarbon containing 1 to 13 carbon atoms, reacted with at least one chain-extending compound selected from the group consisting of diepoxides and compounds which yield the following divalent radicals:



where  $R'$  is a difunctional radical derived from aromatic, heterocyclic, cycloaliphatic or aliphatic hydrocarbons or combinations of them, said fiber having a coating thereon of between about 0.05 and about 6% by weight of said antistatic additive, based on the weight of the finished fiber, said antistatic additive having a melt viscosity of 1,600 to 17,500 centipoises at 100°C.

2. The antistatic fiber of claim 1 wherein  $R$  is a difunctional radical from a lower alkyl aliphatic hydrocarbon compound containing 1 to 6 carbon atoms.

3. The polyamide fiber of claim 1 wherein the ethylene oxide moieties make up about 10 to about 90% of the molecular weight of said tetrol compound and the fiber contains between about 2 to about 10% of the antistatic additive.

4. The polyamide fiber of claim 3 wherein the fiber has a coating thereon of between 0.1 and 3% by weight of said antistatic additive, based on the weight of the finished fiber.

#### EXAMPLE 10

The procedure was that of Example 9 and antistatic additive was similar except that the tetrol compound molecule had 60% ethylene oxide (Tetronic 1506). Carpet samples prepared from this polymer, treated with the instant antistatic additive, and tested in accordance with Examples 2 and 3, showed a static build-up of less than 0.5 K.V.

#### EXAMPLE 11

Ninety-four parts of polyhexamethylene adipamide and six parts of the antistatic material of structure of Example 1 are melt blended by mixing the additive with the molten polyamide at about 285°C. The melt is extruded from a spinneret and the fibers are drawn as described in Example 2. Carpet samples prepared from this fiber, treated with the antistatic additive of Example 9, and tested in accordance with Examples 2 and 3, showed a static build-up of less than 0.5 K.V.

#### DISCUSSION

In additional tests it was determined that the molecular weight of the antistatic compound is preferably between about 9,000 and about 50,000, the ethylene oxide moieties desirably making up about 20 to about 80% of the molecular weight of said compound. Preferably, the antistatic compound has a melt viscosity of 1,600 to 17,500 centipoises at 100°C.

50

55

60

65

\* \* \* \* \*